

## UNITED STATES PATENT OFFICE

2,089,189

MANUFACTURE AND USE OF TEXTILE  
THREADS CONTAINING CELLULOSE ACE-  
TATECamille Dreyfus, New York, N. Y., and William  
Whitehead, Cumberland, Md., assignors to  
Celanese Corporation of America, a corporation  
of DelawareNo Drawing. Application May 18, 1935,  
Serial No. 22,175

11 Claims. (Cl. 117—2)

This invention relates to the manufacture of crepe threads and filaments of cellulose acetate or other organic derivatives of cellulose and to the production of fabrics therefrom wherein a 5 plasticizer is employed to cause the filaments of the yarn to compact, stretch, etc. as they are crepe twisted in the presence of steam.

An object of this invention is the economic and expeditious production of threads containing 10 cellulose acetate or other organic derivatives of cellulose which have a high degree of creping power suitable for the production of crepe fabrics. A further object of this invention is the treatment of yarns and the twisting of same to 15 a high degree of twist in such a manner that fabrics having a uniform creping property are produced. Other objects of the invention will appear from the following detailed description.

The term "organic derivatives of cellulose" as 20 used in this application is intended to include the organic esters of cellulose such as cellulose formate, cellulose propionate, cellulose butyrate and other organic esters of cellulose and also ethers of cellulose such as methyl cellulose, ethyl 25 cellulose and benzyl cellulose. Although the invention hereinafter will be specifically described in particular connection with cellulose acetate, it is applicable for use with yarns or threads made of other organic derivatives of cellulose such as 30 have been hereinbefore mentioned.

It has been found that if yarns of cellulose acetate are tightly twisted, especially in the presence of steam, the same may be woven into a fabric which produces a substantial amount of 35 crepe. By this prior process, however, the amount and type of crepe produced are dependent upon a number of conditions, difficult to regulate, that effect the setting of twist, the compactness of the yarn, etc. These varying conditions which influence the type and amount of 40 crepe that the threads will produce cause difficulties in the manufacture of crepe fabrics consisting entirely or substantially of threads of cellulose acetate. By employing this invention, 45 however, many conditions may be disregarded within wide limits and threads that will produce a uniform type of crepe are formed. Furthermore, by employing this invention, the degree and type of crepe produced is governed by fewer 50 variables, which may be easily controlled, such as the amount of twist imparted to the thread, the type and temperature of treatment given to the fabric in the creping bath and such other manual operations.

55 By prior methods of forming crepe fabric from

threads containing cellulose acetate, it was usually necessary to subject the fabric to lengthy treatments or treatments in rope form in heated aqueous soap baths to cause the threads to shrink and buckle the fabric into the crepe 5 pebble. Unless care was exercised, these treatments were apt to result in permanent boil-off creases being formed in the fabric. By employing this invention, however, the buckling of the fabric occurs substantially immediately with the 10 immersion of the same in the heated creping bath. The speed with which the fabric crepes allows for continuous creping treatments and for the fabric to be treated in open width and for very short periods of time, thus greatly reducing 15 the possibility of boil-off creases. A further advantage of this invention is that the fabric is creped by very short treatments with water near the boil. For this reason, it is not necessary to subject the fabric to long periods of treatment 20 in heated baths where the filaments, due to their thermoplastic properties may be softened. The possibility of the stretching of the fabric in localized areas is thereby greatly reduced.

A still further advantage of this invention is 25 that the threads produced in accordance therewith may contain a smaller number of turns per inch of twist than was heretofore necessary to produce a fabric of substantially the same pebble or crepe properties.

In accordance with the present invention highly 30 twisted crepe threads containing filaments of cellulose acetate or other organic derivatives of cellulose are produced from threads or filaments of cellulose acetate or other organic derivatives of 35 cellulose which have incorporated therein a plasticizer, swelling agent or softening agent, etc., by crepe twisting in a single stage and, during the insertion of the crepe twist, steaming the threads. It is of some advantage to have moisture present 40 during the steaming. Thus, during the twisting operation wet steam may be applied to the travelling yarn over at least a portion of that part of its track in which twisting takes place.

By incorporating a plasticizer with the filaments 45 of cellulose acetate it has been found possible to produce crepe threads which yield fabrics exhibiting crepe effects of an excellence hitherto unattained with cellulose acetate crepe threads. Moreover, with this new process there may be 50 produced cellulose acetate crepe threads which have an average strength very much greater than that of cellulose acetate crepe threads produced by a simple twisting operation without the aid of plasticizers being present during the steam 55

treatment and twisting. Further, apart from the great advantage of a strong resultant thread, the twisting operation itself is greatly facilitated in that twisting may be satisfactorily accomplished under conditions of twist and spindle speed which, in the absence of the plasticizer, would give rise to frequent thread breakage and render impossible the insertion of the desired twist or at least lead to a very weak and useless 10 thread.

Prior to the twisting operation, which imparts the high degree or crepe twist thereto, any suitable plasticizer (i. e. solvent, softening or swelling agent, etc.) may be incorporated with the yarns 15 or filaments. The plasticizer may be incorporated in the yarns in amounts up to 10% or more on the weight of the yarns by adding the same to the spinning solution or dope from which the filaments constituting the thread or yarn 20 are formed. However, similar amounts of plasticizer may be added to the formed yarn as a coating. Thus, up to 10% or more of a plasticizer may be added to a solution of cellulose acetate in a volatile solvent and the same extruded 25 through orifices of suitable shape and diameter to form the type of yarn desired. Either the wet or dry method of spinning may be employed. By another modification the plasticizer may be incorporated with the yarn by applying the same 30 as a coating to the yarn after the yarn has been formed. The plasticizer may be applied to the yarn as the sole constituent of the coating or along with a suitable lubricant and/or thinner and may be applied at the metier as the yarns 35 are formed or during any subsequent winding operation prior to imparting twist thereto. The coating material may consist of from 5 to 100 parts of a plasticizer and 95 to no parts of lubricating material. The lubricating material 40 containing the plasticizer may be applied to the yarn while the yarn is travelling as at its formation, or during any winding operation, by causing the yarn to contact with a wick or roller that dips into a mixture or solution containing 45 same or by any other furnishing device.

Any suitable plasticizer may be employed and by that term is meant the high boiling solvents, swelling agents or softening agents, etc. for cellulose acetate, as for example: the aryl sulfonamides such as para ethyl toloul sulphonamide, the alkyl phthalates such as dimethyl phthalate, the di-alkyl tartrates such as di-butyl tartrate, the alkoxy esters of polybasic organic acids such as diethoxy ethyl phthalate, the poly-55 basic organic acid esters of the monoalkyl ethers of polyhydric alcohols such as diethylene glycol ethyl ether ester of phthalic acid, the alkyl esters of phosphoric acid such as tri-ethylglycol phosphate, the aryl esters of phosphoric acid such 60 as tri-cresyl phosphate and the mixed alkyl and aryl phosphates such as ethylglycol di-cresyl phosphate. Mixtures of two or more of the above may be employed.

The yarns to be formed into crepe threads may 65 consist of substantially continuous filaments of cellulose acetate or they may contain discontinuous filaments of cellulose acetate, the length of which may vary within wide limits. Where discontinuous filaments are employed, they may 70 be formed into yarns by the cotton, wool or silk method of spinning or by breaking continuous lengths in the yarn. For example, the threads may be those spun from a mass of discontinuous filaments or those prepared in the manner de-75 scribed in co-pending U. S. application S. No.

726,264, filed May 18, 1934. The yarns may be formed wholly of filaments or fibers of cellulose acetate or the yarns may also contain filaments and/or fibers of other materials, for instance, wool, cotton, silk, other organic derivatives of cellulose, regenerated cellulose, etc. If other fibers or filaments are employed with the filaments or fibers of cellulose acetate, they may be incorporated with the yarns by forming the 10 yarns by a wool, cotton or silk method of spinning, or by doubling a yarn from two or more yarns, one of which contains cellulose acetate.

If desired, the filaments of the yarns to be formed into the crepe threads may contain water-insoluble compounds, such as compounds of 15 pigment-like character, in such form as materially to modify the lustre of the filaments (e. g. barium sulphate or titanium dioxide), or loading metal compounds, for example, tin compounds. 20

In carrying out the new process, twisting may be effected on a device of the kind in which the thread is drawn off over the end of a rotating package through a guide fixed preferably substantially in line with the axis of rotation of the 25 package and is thereafter wound on a bobbin or the like, the thread being passed, on its way from the guide to the bobbin, through steam. In this way the thread is subjected to the action of the steam during the actual application of a 30 substantial amount of the twist, or to the action of both steam and moisture if it is passed through steam under such conditions that moisture is present. On the other hand, any other suitable crepe twisting device may be employed 35 in conjunction with steaming. For example, a ring twister may be used for the crepe twisting of thread consisting of discontinuous cellulose acetate filaments. Also as an example of an efficient type of crepe twisting device reference 40 may be had to U. S. application S. No. 19,052, filed April 30, 1935. It is preferable that the twisting mechanism, the thread guides, the supply package, the take-up package and the steaming device be so arranged that the twist resulting 45 from the rotation of the package or twisting mechanism is at least partly inserted while the thread is under the influence of steam. 50

Steaming may conveniently be effected by allowing the thread to pass through a suitable chamber supplied with steam preferably under such conditions that moisture is present. The chamber may be provided with small holes, top and bottom, to permit of passage of the thread, and also with a steam inlet. The size of the 55 chamber may be sufficient to afford the thread the requisite length of travel in the steam. Alternatively, a chamber having a smaller diameter may be used, in which case the chamber may be provided with hollow nipples communicating 60 therewith and through which the yarn passes, the nipples being of sufficient size to provide, together with the size of the chamber, the requisite length of travel in the steam.

The presence of the desired moisture may be 65 assured by supplying wet steam to the steaming device and/or by arranging for the condensation of steam to supply the requisite moisture. Wet steam may be conveniently produced by passing steam through water at suitable velocity, for instance, small traps for condensed water may be provided at suitable intervals in the steaming chamber and steam injected therethrough by means of small pipes or orifices. Another method of ensuring the presence of moisture is to wet 70 75

the thread with water. For example, the bobbins of thread may be wetted before the twisting operation or, better, water may be applied to the thread by means of a wick or other device after the thread leaves the spindle and prior to its entering the steaming device.

Steam at slightly above atmospheric pressure, or at a pressure of 1 or more millimeters of water is most conveniently employed. If desired, however, the steaming may be effected with steam at any desired super-atmospheric pressures, e. g., steam at 10-25 lbs. per square inch.

A steaming treatment of relatively short duration, such as may be secured by passing the yarn 15 at a speed of from 2 to 10 metres per minute through say from 1" to 3" of steam, has been found to give satisfactory results. Lengthier treatments may, however, be employed, for example, the yarn may be passed at the said speeds 20 through 6 to 12" or more of steam.

The cellulose acetate filaments of the threads when the threads have incorporated therewith a plasticizer or softener very readily undergo stretching when the threads are twisted under 25 the influence of the steam and moisture. The amount of stretch may be measured by comparing the original thread denier with the final thread denier (after untwisting). It has been found that when a cellulose acetate thread is 30 crepe twisted by the new process involving treatment with a plasticizer and steaming during twisting so as to produce a crepe thread of good strength and creping properties, the denier of the resultant thread is, in general, owing to imparted stretch, less and even substantially less than if the thread is simply crepe twisted without such treatments. The stretch imparted to the filaments of the thread during the twisting operation may, for example, be of the order of 35 40 5-25% of their original length, and particularly 10-20%. The degree of stretching of the filaments of the thread may be such that the final denier of the crepe twisted thread is not much in excess of or is even the same or less than the 45 denier of the thread prior to twisting. For example, the stretch may be such that the denier of the crepe twisted thread is from 95 to 115%, 120% or 125%, or more, particularly 100 to 110% of that of the thread before crepe twisting, especially in case of threads having an original denier 50 of 200 or less. In the case of heavier threads, i. e., those having a denier above 200, the denier increase may be greater and still good crepe effects attained.

55 The degree of twist applied in accordance with the new process may vary within wide limits but is, in general, less than that formerly required to produce the same type of crepe in the fabric. The process, moreover, permits of the insertion 60 of twists which are impossible of attainment without the steaming in the presence of a plasticizer, owing to the breakage of the thread. This is important since it enables crepe fabrics having very pronounced yet uniform crepe effects to be produced. The crepe figure can be regulated according to requirements. The degree of twist desirable in any particular case depends upon a number of factors, including the precise effects required, and the denier and number of filaments 65 70 in the thread. For example, threads of 150 denier may be twisted to about 55 to 75 or more turns per inch, while 100 denier threads may be twisted to about 60 to 100 or more turns per inch. Proportionate twists may be used in case 75 of threads of other deniers.

By the new process highly twisted cellulose acetate crepe threads may be produced in which the filaments are extremely closely packed. For example, as appears from a microscopic examination of the cross-sections of yarns twisted in accordance with this invention, the filaments are 5 squeezed together into substantially as close contact as possible, causing some distortion of the cross-section of at least some of the filaments thereof. Further, as appears from a microscopic 10 examination of the cross-sections of threads twisted in accordance with this invention, filaments that formerly were bulbous in character are squeezed together so closely that they assume a shape, not necessarily bulbous, to more nearly 15 fill up the circle of the cross-section. The filaments, however, are not stuck together nor adhered to each other and they can be separated upon untwisting into individual filaments. The threads produced in accordance with the present 20 invention have a specific gravity of at least 85% of that of a solid thread.

The highly twisted crepe threads may be incorporated in the fabrics in various ways, for example, the weft alone may be wholly or partially composed of such threads or the warp may also contain them. Valuable fabrics may be produced by employing in the warp, threads of relatively low twist and in the weft both crepe threads having a left-hand twist and crepe 30 threads having a right-hand twist, pairs of threads of left-hand twist alternating with pairs of threads of right-hand twist.

If desired, the cellulose acetate crepe threads 35 may be associated in the fabrics with highly twisted crepe threads of other materials, e. g., of natural silk or regenerated cellulose, or threads of artificial silk produced by other processes. Where the fabrics contain threads of low twist, these may wholly be of cellulose acetate or wholly 40 or in part of other materials, e. g., natural silk or regenerated cellulose.

After the yarns or threads have been formed into a fabric, if said threads or any of said threads have been treated with very active and 45 large amounts of plasticizers such as di-ethylene glycol, etc., the fabric, to produce the best creping effect, should be scoured in water below 95° C. or dry cleaned to remove a part or all of the plasticizer present. If a large amount of very 50 active plasticizer is present in the thread during the creping, the creping forces release themselves without buckling the yarn. When the fabric is first scoured cold or dry cleaned with an organic solvent for the plasticizer, however, it crepes 55 heavily and produces a very uniform fabric in the subsequent heated creping bath. When smaller amounts or less active plasticizers are employed, such as tricresyl and triphenyl phosphate, etc., the fabric need not be scoured cold 60 prior to the treatment in the hot bath to produce the crepe effect on the fabric. The action of the various plasticizers employed may be tested to ascertain which, if any, and to what extent the same should be scoured from the fabric in the 65 cold before placing the fabric in the heated bath to develop the crepe effect and to buckle the threads in the fabric. Fabrics containing highly twisted crepe threads prepared in accordance with this invention may be scoured in the cold 70 bath to remove a part or all of the plasticizer employed for the twisting operation, if the same is necessary, and then subsequently be scoured, for example, in the manner adopted in connection with fabrics comprising highly twisted yarn 75

of natural silk. Enhanced crepe effects may be obtained by employing scouring or other aqueous crepe baths at or near the boiling point. The fabric made in accordance with this invention 5 may be caused to crepe by immersing the same in a bath, containing up to 10 grams or more per litre of soap, that is maintained at about 95° to 105° C. However, by employing certain plasticizers, the temperature of the creping bath may 10 be considerably lower. The period of treatment in the heated bath may be from a fraction of a minute, where yarns contain a plasticizer, to 5 or 30 or more minutes where the plasticizer has been removed or is present as a coating on the 15 yarn. The delustering effect of all high temperature scouring baths upon fabrics containing threads of lustrous cellulose acetate may be minimized by incorporating therein salts or sugars.

An important characteristic of fabrics exhibiting 20 crepe effects produced in accordance with this invention is that unlike crepe fabrics heretofore produced, they do not shrink substantially when washed or otherwise treated with aqueous liquids, nor do they tend to develop spots when 25 subjected locally (such as by rain) to aqueous liquids. Therefore, garments or other articles made of such fabric may be laundered in the ordinary way without recourse to dry cleaning.

As illustrations in describing this invention and 30 not as limitations, the following examples are given:

*Example I*

A spinning solution is formed by mixing substantially 25 parts of acetone-soluble cellulose acetate, 75 parts of acetone and 0.5 part of di-40 ethylene glycol. This solution is spun into filaments by the dry method of spinning. The yarn as formed is lubricated with olive oil, or other 45 yarn lubricant, and subsequently twisted to a crepe thread by imparting thereto, in the presence of steam, a twist of about 70 turns per inch. This yarn is woven into a fabric and then washed in water below 45° C. in the presence of a soap 50 solution sufficient to remove substantially 75% of the di-ethylene glycol present in the yarn. The fabric is then treated for 10 minutes in an aqueous bath maintained at 99° C. The fabric produced has a heavy and uniform crepe effect produced thereon, which crepe effect is spot-proof and substantially free from further shrinkage upon treatments in aqueous or other cleaning baths normally met with in the use of the fabric.

*Example II*

55 A spinning solution is formed by mixing substantially 25 parts of acetone-soluble cellulose acetate, 75 parts of acetone and 1.5 parts of tricresyl phosphate. This solution is spun by the dry method of spinning into a yarn, which yarn is lubricated with a suitable yarn lubricant. The 60 yarn so produced is twisted, in the presence of steam, to a crepe thread having approximately 70 turns per inch. This thread is woven into a fabric and same immersed in an aqueous bath 65 maintained at a temperature of above 80° C. for about 1 minute. The fabric produced has a heavy crepe effect, is exceptionally uniform and strong. This material is spot-proof and does not 70 materially shrink upon further treatment in cleansing baths or solutions.

*Example III*

A yarn of cellulose acetate is caused to contact 75 with a furnishing device which applies thereto

a coating of tricresyl phosphate. The amount of coating applied to the yarn may be any suitable amount, for example, from 1 to 5% or more based on the weight of the yarn. This yarn is twisted to a crepe thread in the presence of steam, 5 such that approximately 70 turns per inch are inserted therein. The threads are woven into a fabric and the fabric treated in a hot bath maintained at above 80° C. for a period of from 10 to 20 minutes. The fabric produced is similar in 10 all respects to that produced by Example II. In place of a coating of tricresyl phosphate the yarn may be coated with 2% or 3% on the weight of the yarn of a 50-50 mixture of dibutyl tartrate and olive or castor oil. This yarn need not be 15 scoured in cold water prior to creping.

In the above specification and in the appendant 20 claims the term "plasticizer" is intended to include within its scope any reagent as explained above which has a swelling, softening or slight 25 solvent action upon the filaments containing cellulose acetate or other organic derivatives of cellulose at above room temperature. This term is intended to include plasticizers, softeners and swelling agents.

It is to be understood that the foregoing detailed description is merely given by way of illustration and many alterations may be made therein without departing from the spirit of our invention. 30

Having described our invention, what we desire to secure by Letters Patent is:

1. Process for the production of highly twisted 35 crepe thread of filaments containing an organic derivative of cellulose, which comprises incorporating a plasticizer with the thread, steaming the thread and crepe twisting the thread while it is subjected to the action of the steam.

2. Process for the production of highly twisted 40 crepe thread of filaments containing an organic derivative of cellulose, which comprises incorporating a plasticizer with the thread, crepe twisting the thread of filaments in a single stage and steaming the thread during the actual insertion of the crepe twist. 45

3. Process for the production of highly twisted 50 crepe thread containing filaments of an organic derivative of cellulose, which comprises incorporating a plasticizer with the thread containing filaments of an organic derivative of cellulose, crepe twisting said thread and, during the actual insertion of the crepe twist, steaming the thread under such conditions that moisture is present. 55

4. Process for the production of highly twisted 60 crepe thread of filaments containing cellulose acetate which comprises incorporating a plasticizer with the thread, crepe twisting the thread of filaments in a single stage and steaming the thread during the actual insertion of the crepe twist. 65

5. Process for the production of highly twisted 70 crepe thread containing filaments of cellulose acetate which comprises incorporating a plasticizer with the thread containing filaments of cellulose acetate, crepe twisting said thread and, during the actual insertion of the crepe twist, steaming the thread under such conditions that moisture is present. 75

6. Process for the production of highly twisted 80 crepe thread of filaments of cellulose acetate which comprises incorporating a plasticizer with a thread of filaments of cellulose acetate, crepe twisting said thread in a single stage and, during the actual insertion of the crepe twist, steaming the thread under such conditions that moisture 85

is present and stretching the filaments of the thread from 5 to 25% of their original length.

7. Process for the production of highly twisted crepe thread of filaments of cellulose acetate which comprises incorporating a plasticizer with a thread of filaments of cellulose acetate, crepe twisting said thread and, during the actual insertion of the crepe twist, steaming the thread and stretching the filaments thereof.

10 8. Process for the production of highly twisted crepe thread of filaments of cellulose acetate which comprises incorporating a coating containing an aryl phosphate with a thread of filaments of cellulose acetate, crepe twisting said thread and steaming the thread during the actual insertion of the crepe twist.

9. Process for the production of highly twisted crepe thread of filaments containing a cellulose ether, which comprises incorporating a plasticizer

with the thread, crepe twisting the thread of filaments in a single stage and steaming the thread during the actual insertion of the crepe twist.

10. Process for the production of highly twisted crepe thread of filaments of a cellulose ether, which comprises incorporating a plasticizer with a thread of filaments of a cellulose ether, crepe twisting said thread in a single stage and, during the actual insertion of the crepe twist, steaming the thread under such conditions that moisture is present.

11. Process for the production of highly twisted crepe thread of filaments containing cellulose acetate, which comprises incorporating a plasticizer with the thread, steaming the thread, and crepe twisting the thread while it is subjected to the action of steam.

CAMILLE DREYFUS.  
WILLIAM WHITEHEAD.